

106. COMPOSITIONS,  
COATING OR PLASTIC

Cross Reference

Examiner

98

March 8, 1927.

1,620,312

H. B. ABBOTT

COMPOSITION OF MATTER ADAPTED TO BE USED FOR BUILDING MATERIAL

Filed Oct. 26, 1925



Inventor

Harvey B. Abbott

106.  
98

Patented Mar. 8, 1927.

1,620,312

XR

## UNITED STATES PATENT OFFICE.

HARVEY B. ABBOTT, OF GLASSBORO, NEW JERSEY.

### COMPOSITION OF MATTER ADAPTED TO BE USED FOR BUILDING MATERIAL.

Application filed October 26, 1925. Serial No. 65,032.

This invention relates to a composition of matter for building material and a building block formed therefrom and it consists in the novel features hereinafter described and 5 claimed.

An object of the invention is to provide a composition of matter which may be advantageously and economically used for forming concrete block and using soft coal cinders as an ingredient of the composition.

A further object of the invention is to provide a composition which may be used in a block and having qualities which will tenaciously hold stucco and plaster to the surfaces of the block when the block is laid in a wall.

A further object of the invention is to provide a block which is light in weight and easy to handle.

20 A further object of the invention is to provide a composition which will give the block maximum tensile strength.

A further object of the invention is to provide a composition which utilizes a practical- 25 ly waste material, thus reducing the cost of producing the block.

In the accompanying drawing:—

Figure 1 is a top plan view of a building block formed from my composition of matter.

Figure 2 is a side elevational view of the block.

Figure 3 is an end elevational view of the same.

35 The composition of matter consists of soft coal cinders, sand and cement. These ingredients are mixed and are supplied with a suitable quantity of water to effect an intimate mixture and tenacious concrete adhesion.

40 The soft coal cinders are first ground whereby they are reduced to grains of approximately uniform size. The grain of the cinders will retain a certain amount of the residuum of the bitumen originally contained 45 in the coal and at the same time the cinders in the ground form will be sharp enough to afford anchorage for the cement. The bitumen retained in the grains of the cinders 50 will be sufficient to add waterproof qual-

ties to the composition, toughness and to a limited degree pliability.

To form a block weighing about 38 pounds avoirdupois the ingredients are mixed substantially in the following stated propor-

tion:—  
19 pounds avoirdupois ground bituminous cinders.

12 $\frac{1}{2}$  pounds avoirdupois, sand.  
6 $\frac{1}{2}$  pounds avoirdupois, cement.

1 $\frac{1}{3}$  quarts, liquid measure, water.

These ingredients are mixed and the operation relating to the construction and manufacture of the block is conducted in the same general manner as the manufacture of 65 cement concrete block products.

As illustrated in the drawing, the body of the block 1 is hollow and the surfaces of the body are provided with a vast number of pockets 2 indicated by the dots upon the surfaces of the body of the block. These pockets are formed by the evaporation of the water from the composition during the molding of the block and these pockets are lined with the mixed cement and bitumen of the 75 soft coal cinders. These pockets constitute a vast number of minute cavities to which stucco and plaster will cling when applied to the block in the wall. They also afford anchorage cavities for mortar.

The block is provided at its end surfaces with vertical grooves 3 which are spaced from each other and which extend from the lower to the upper side surface of the block. The block is further provided at its end surfaces with horizontal grooves 4 located between the grooves 3 and spaced from the grooves 3 and from each other. The grooves 3 and 4 are adapted to receive and hold tenons of mortar when the block is laid in a 80 wall, thus preventing lateral movement of the block in any direction. The surfaces of the grooves 3 and 4 are also provided with pockets 2 which serve as additional anchorage cavities for the mortar.

Having described the invention, what is claimed is:

1. The composition of matter for building blocks consisting of proportions by weight of ground soft coal cinders to the quantity 100

of approximately 19 parts, sand to the quantity of approximately 12 $\frac{2}{3}$  parts, cement to the quantity of approximately 8 $\frac{1}{3}$  parts, water to the quantity of approximately 2 $\frac{2}{3}$  parts.

a uniform size in the quantity of approximately 19 parts, sand in the quantity of approximately 12 $\frac{2}{3}$  parts, cement in the quantity of approximately 6 $\frac{1}{3}$  parts, and water in the quantity of approximately 2 $\frac{2}{3}$  parts.

10

2. The composition of matter for building blocks consisting of proportions by weight of soft coal cinders ground to substantially

In testimony whereof I hereunto affix my signature.

HARVEY B. ABBOTT.